

No. 842,254.

PATENTED JAN. 29, 1907.

A. SCHWARZ.

PROCESS FOR THE ELECTROLYTIC REFINING OF METALS.

APPLICATION FILED FEB. 6, 1904.

Fig. 1



Fig. 3



Fig. 2



Fig. 4



WITNESSES:

Grace D. Hesley.  
May S. Arvey.

INVENTOR

Alfred Schwarz  
BY  
Charles S. Jones  
his ATTORNEY

# UNITED STATES PATENT OFFICE.

ALFRED SCHWARZ, OF NEW YORK, N. Y.

## PROCESS FOR THE ELECTROLYTIC REFINING OF METALS.

No. 842,254.

Specification of Letters Patent.

Patented Jan. 29, 1907.

Application filed February 6, 1904. Serial No. 192,444.

*To all whom it may concern:*

Be it known that I, ALFRED SCHWARZ, a subject of the Emperor of Germany, and a resident of the borough of Manhattan, city, county, and State of New York, have invented certain new and useful Improvements in the Process for the Electrolytic Refining of Metals, of which the following is a specification.

10 Heretofore in the electrolytic extraction or refining of metals the usual practice has been to subject the ore to several preliminary operations, depending upon the nature and character of the ore, and to smelt the concentrates into mattes to be used as anodes.

The present invention has been devised by me to deal directly with the ores in the form of concentrates, the object being to simplify present methods in the manner more fully 15 hereinafter described and claimed.

In the accompanying drawings, Figure 1 is a face view of an anode base; Fig. 2, a similar view of the base filled with concentrates; and Figs. 3 and 4, respectively, are transverse 20 sectional views on the lines 3 3 and 4 4 of Figs. 1 and 2.

Similar reference-numerals indicate similar parts throughout the several views.

The ore to be refined is first crushed to a 25 convenient size for handling and then concentrated in any well-known or suitable manner to separate the values from the gangue, which is essentially silicious. The concentrates without further treatment are 30 collected and compressed by any suitable means into solid masses or cakes of a form and size that will adapt them to be used as anodes in an electrolytic refining-tank. For this purpose an adhesive may be employed, 35 if desired, to make a compact mass and to retain the mass in proper shape and condition for handling.

Owing to the nature of the concentrates and of the liability of the compressed masses 40 to disintegrate, I support such masses in a suitable framework of an insoluble conductive material somewhat after the manner of the plates for secondary batteries. For example, a framework of wood divided into 45 compartments or sections by cross-pieces may be employed, the concentrates being compressed into the open spaces, so as to be exposed to the action of the solution. Such framework will be covered with a suitable 50 conductor in contact with the concentrates to properly deliver the electric current. A

suitable form of anode is shown in the drawings, in which the numeral 1 designates a frame of an insoluble conductive material. This frame is divided by transverse and longitudinal pieces 2 and 3 into sections or compartments 4, into which the concentrates are compressed in the form of cakes or masses 5, or the entire framework may be made of a conductive insoluble material having upon 55 its surface a number of pieces projecting into the compressed mass of concentrates to retain such mass in position. Other expedients will readily suggest themselves by which the concentrates may be properly supported during the electrolytic action, and I only mention the above as simple and inexpensive means for the purpose.

In applying my process to the refining of copper ores I employ a solution of copper sulfate containing a small percentage of free sulfuric acid, and any suitable cathode, preferably of copper, and any economical means for generating electricity. With such a solution the copper contained in the anode will 60 be dissolved and deposited on the cathode, according to well-known principles. The electrolytic action is so controlled that any silver which may be contained in the concentrates is not deposited and may be recovered from 65 the solution by any well-known precipitation method or otherwise. Any gold that may be present in the anodes falls to the bottom of the tank in the form of slime and may be recovered by known methods.

An advantage of importance attaching to the invention above described is that the expense of smelting the ore into mattes is obviated and a simple method provided for the direct handling of the concentrates. As a 70 specific example I may take a chalcopyrite ore and concentrate the same by any well-known method. The concentrates after collection are compressed into a frame, as above described, and suspended in an electrolytic 75 tank containing sulfuric acid or a copper sulfate solution having an excess of acid. The copper contained in the concentrates will 80 pass into solution and be deposited on a suitable cathode under a current density of three to five amperes per square foot and approximately one to one and one-half volts. The iron contained in the concentrates will 85 go into solution in the form of a sulfate, and after all the copper has been dissolved and deposited the solution may be treated for the separation and recovery of the iron in 90

the form of an oxid and the sulfuric acid. The anode-frame may then be used to receive a fresh charge of concentrates. The slimes collected in the bottom of the tank may be treated for the recovery of any gold, silver, antimony, or other metal contained in them.

What I claim, and desire to secure by Letters Patent, is—

The process of depositing a metal from its ore consisting in compressing the concentrates of the ore to be treated into solid masses or cakes and supporting such masses

in a framework of an insoluble conductive material, and then subjecting said anodes to the action of a current in an electrolytic bath.

In testimony whereof I have hereunto signed my name in the presence of two subscribing witnesses.

ALFRED SCHWARZ.

Witnesses:

E. H. PATTON,  
CHARLES S. JONES.